

## UNITED STATES PATENT OFFICE.

SIMON JOSEPH LUBOWSKY, OF JERSEY CITY, NEW JERSEY.

## METHOD OF PRODUCING METALLIC TITANIUM OR ITS ALLOYS.

No Drawing.

Application filed May 3, 1923. Serial No. 636,458.

*To all whom it may concern:*

Be it known that I, SIMON J. LUBOWSKY, a citizen of the United States, and a resident of Jersey City, in the county of Hudson and State of New Jersey, have invented a certain new and useful Method of Producing Metallic Titanium or Its Alloys; and I do hereby declare the following to be a full, clear, and exact description of the invention, such as will enable others skilled in the art to which it appertains to make and use the same.

In my co-pending application Serial No. 636,457, filed of even date herewith, I stated that I had found that titanium oxide, preferably rutile, heated under certain conditions, viz, in a non-oxidizing atmosphere at a temperature from 800° C. to 1,000° C., is converted to a black or gray-black material having the property of thermal and electrical conductivity. I now find that these properties can be utilized and assist greatly in the reduction of these oxides to lower oxides or to the metal itself. Many experimentors have tried, without success, to produce, for instance, metallic titanium from its oxides by ordinary reduction methods, such as the use of any reducing agent (aluminum, carbon, silicon, manganese, magnesium, sodium, calcium, etc.), either with or without the use of the electric furnace; and I find that the new properties of this titanium oxide render it suitable for reduction by these methods; for instance, I have found it entirely practical to produce metallic titanium from this converted titanium oxide by means of the well known aluminothermic reaction. In this work, I have proceeded as follows:

40 I have made a thermit by mixing ground, converted titanium oxide with aluminum in the degree of fineness regularly used in thermit operations in the proportion of 100

parts of oxide to 45 parts of aluminum. I have placed this in a crucible in which the 45 contents could be highly heated, and after this heating, have applied the regular ignition powder to initiate the thermit reaction. I have found that the reaction propagates rapidly throughout this heated mass and 50 results in the production of a regulus of metallic titanium and the usual aluminothermic slag. Parallel experiments performed with unconverted rutile and titanium dioxide proved unsuccessful. 55

It is obvious that the proportions of oxide to aluminum may be varied considerably from those given above and that flux, as well as accelerators, may be added to improve the efficiency of the production. It is further obvious that, if the proportion of aluminum used is increased, an alloy of the titanium with aluminum may be formed, and that by the addition of metals, oxides, thermits or other substances, other desired 60 alloys may be produced. It is further obvious that instead of carrying on this reaction in a crucible, the reaction may be produced in an electric furnace using either aluminum or one of the other reducing 70 agents, the electric arc being sufficient, of course, to both preheat the material and initiate the reaction.

What I claim is:

1. The method of producing metallic titanium which comprises treating a gray-black oxide of titanium by the application of heat in the presence of metallic aluminum. 75

2. The method of producing metallic titanium which comprises effecting the aluminothermic reaction between a gray-black oxide of titanium and metallic aluminum. 80

In testimony whereof I affix my signature.

SIMON JOSEPH LUBOWSKY.